

# United States Patent Office

3,133,006  
Patented May 12, 1964

1

3,133,006

## ACID NICKEL PLATING BATH

Barnet D. Ostrow, 125 Redwood Drive, and Fred I. Nobel,  
75 Fern Drive, both of Roslyn, N.Y.  
No Drawing. Filed May 28, 1962, Ser. No. 197,860  
6 Claims. (Cl. 204—49)

The present invention relates to the electrolytic deposition of nickel, and it is directed primarily to the production of bright, smooth and lustrous deposits.

Previously, acid nickel plating baths were modified by the introduction therein of additives intended to produce brightness of nickel deposits. Among such additives were various types of substances in conjunction with aromatic and aliphatic sulfonates, sulfonamids and sulfonimids. These prior suggested substances included alkynes, alkenes, amines, alkyne amines, and alkene amines. Such substances had in the molecule an allylic or vinyl group only, an acetylenic group only, or an active amino group only. It has also been proposed to incorporate compounds having in the same molecule an amino and an allyl or vinyl group.

While some addition agents accomplished this purpose in some degree, they did not contribute to superior leveling coupled with the ease of control. Also, because of the high concentration of these compounds that were necessary to produce the desired brightness and leveling the ductility was impaired. In some cases as with the alkynols the deposit has a marked tendency to "skip plate," i.e. to prevent deposition of nickel at the low current densities.

The present invention has among its objects to introduce additives, for the above purpose, into aqueous acid nickel plating baths, which will result in excellent leveling of the deposit.

It is also among the objects of the invention to provide a bath for the purpose described which will reduce the low current density skip plate in the deposited film of nickel.

In practicing the invention, there is provided the usual aqueous acid nickel plating bath and there is incorporated therein an additive which consists of at least one compound which contains in the same molecule an amino, an alkyne, and an alkene group. Substances having these three groups impart superior leveling characteristics to the bath, with a substantial improvement in low current density characteristics of the nickel deposit. Relatively small amounts of these substances are very effective, and they do not impair the ductility of the deposit.

These substances have the following structural formulae:



wherein  $R_1$  is an alkene group;  $R_3$  is an alkyne group;  $R_2$  and  $R_4$  are alkene, alkyne, H,  $CH_3$ ,  $C_2H_5$ ,  $C_3H_7$ , phenyl and naphthyl and  $X$  is an acid group, such as halogen,  $SO_3H$ , or  $PO_4$ . Compounds (C) and (D) may be quaternized.

While alkene and alkyne carbon chains up to 8 carbon

2

atoms may be present in the molecule, at present the lower carbon chains are considered to be more desirable. Together with the substances of the invention, the structural formulas of which are given above, other acetylenic compounds may be incorporated into the bath, thus employing a mixture of unsaturated compounds.

The structural formulas given below are illustrative of the substances included in the invention.



The essence of the invention lies in the structures of the additives in which there are combined in a single molecule, the amino, alkyne and alkene radicals. The deposits resulting from baths containing these additives have high lustre and are smooth with excellent leveling. In addition, the deposits do not exhibit low current density greyness which often occurs when additives such as amines or polyamines are used in the bath.

Compounds of the present invention may be used singly or in mixtures or in the absence of other types of additives. They may be used in standard Watts baths, all chloride baths, or high chloride baths. Improved results are obtained where there is incorporated therewith in the bath a sulfonic acid, sulfonamid or sulfonimid.

Typical standard nickel baths which are employed in the invention are as follows in grams per liter.

Watts bath:

|                      |         |
|----------------------|---------|
| $NiSO_4 \cdot 7H_2O$ | 100-400 |
| $NiCl_2 \cdot 7H_2O$ | 5-80    |
| Wetting agents       | 0-1     |
| Boric acid           | 5-60    |
| All chloride bath:   |         |
| $NiCl_2 \cdot 7H_2O$ | 50-200  |
| Boric acid           | 0-50    |
| Wetting agent        | 0-1     |

Among typical wetting agents are sodium lauryl sulfates, sodium 2-ethyl hexyl sulfate, and sodium octyl sulfonic acid. The range of pH is from 2.5 to 4.5 in usual practice.

The following are specific examples of baths according to the invention which are employed to obtain bright, level and ductile deposits; the amounts being in grams per liter of aqueous solution:

|                                   | 1   | 2    | 3   | 4   | 5    |
|-----------------------------------|-----|------|-----|-----|------|
| Nickel Sulfate                    | 300 | 300  | 250 | 300 | 200  |
| Nickel Chloride                   | 45  | 45   | 75  | 60  | 120  |
| Boric Acid                        | 45  | 45   | 40  | 35  | 40   |
| Saccharin                         |     | 1.0  |     |     |      |
| Bromo Benzene Sulfonate           | 8   |      |     |     |      |
| 1,5-Benzene Disulfonate           |     |      |     |     | 15   |
| Vinyl Benzene Sulfonate           |     | 0.6  |     |     |      |
| Sodium Allyl Sulfonate            |     |      | 0.5 |     |      |
| Sodium Benzenaldehyde Sulfonate   | 2   |      |     |     |      |
| Dibenzeno sulfonamid              |     |      | 1.5 |     |      |
| Allyl sulfonamid                  |     |      |     | 1.5 | 0.5  |
| 3-Dialyl amino propyne-1          |     |      |     | .01 |      |
| Triallyl propargyl amine chloride |     | 0.04 |     |     |      |
| 1-Allyl 3-amino dipropyne         | .06 |      |     |     |      |
| 1-Allyl amino 2-butyne            |     |      |     |     | 0.07 |
| Allyl propargyl amine             |     |      | .03 |     |      |
| pH                                | 4.2 | 4.3  |     | 3.6 | 4.0  |
| Temp., ° F                        | 135 | 140  | 140 | 135 | 155  |

Examples of amino vinyl acetylenic compounds are as follows:

Allyl propargyl amine  
Diallyl propargyl amine  
Triallyl propargyl amine  
Vinyl propargyl amine  
Allyl dipropargyl amine  
Divinyl propargyl amine  
Triallyl propargyl amine hydrochloride  
Bis 1,4-allyl amine 2-butyne  
Bis 1,4-diallyl amine 2-butyne  
Bis 1,4-triallyl amine 2-butyne

The following sulfonic acids may be incorporated in the bath with the principal additive; they may be in the form of salts, such as of nickel, sodium, magnesium, etc.

Benzene sulfonic acid  
Di-benzene sulfonic acid  
Vinyl benzene sulfonic acid  
Allyl benzene sulfonic acid  
Bromo benzene sulfonic acid  
1,5-naphthalene disulfonic acid  
1,3,6 naphthalene trisulfonic acid

Among the sulfonamids and sulfonimids which are suitable are the following:

Saccharin Na salt  
Benzene sulfonamid  
Dibenzene sulfonamid  
Allyl sulfonamid

The baths of the invention may be operated over a wide range of concentration, pH, and current densities. A pH range of 3.0 to 4.8 is typical. The concentration of the additive may vary from about .001 to .50 gram per liter when used with cooperating sulfo oxygen type materials. The concentration of the sulfo oxygen will generally determine the concentration of the alkene-alkyne amine. When used alone, the concentration of the alkene-alkyne amine generally ranges from about .001 to 1.0 gram per liter.

These baths may be operated with or without mechanical or air agitation. When air is used, a compatible low-foaming or non-foaming type of wetting agent is employed in the bath. The invention may be used in all sulfate baths, that is baths substantially free from chlorides; and it is suitable for sulfamate baths also.

We claim:

1. An aqueous acid nickel electroplating bath having incorporated therein an amine having as substituent groups an alkene and an alkyne radical attached to nitrogen and having the following structural formula:



wherein  $R_1$  is an alkene group and  $R_4$  is a radical taken

from the class consisting of alkene, alkyne, H, and lower alkyl, and  $R_3$  is alkyne.

2. An aqueous acid nickel electroplating bath having incorporated therein an amine having as substituent groups an alkene and an alkyne radical attached to nitrogen and having the following structural formula:



wherein  $R_1$  is alkene,  $R_3$  is alkyne, and  $R_2$  and  $R_4$  are taken from the class consisting of alkene, alkyne, H, and lower alkyl, and X is an acid group.

3. An aqueous acid nickel electroplating bath having incorporated therein an amine having as substituent groups an alkene and an alkyne radical attached to nitrogen and having the following structural formula:



wherein  $R_1$  is alkene,  $R_3$  is alkyne, and  $R_2$  and  $R_4$  are taken from the class consisting of alkene, alkyne, H, and lower alkyl.

4. An aqueous acid nickel electroplating bath having incorporated therein an amine having as substituent groups an alkene and an alkyne radical attached to nitrogen, and having the following structural formula:



wherein  $R_1$  is alkene,  $R_3$  is alkyne, and  $R_2$  and  $R_4$  are taken from the class consisting of alkene, alkyne, H, and lower alkyl.

5. A nickel plating bath according to claim 3, characterized in that said compounds are quaternized.

6. A nickel plating bath according to claim 4, characterized in that said compounds are quaternized.

#### References Cited in the file of this patent

#### UNITED STATES PATENTS

|           |         |               |
|-----------|---------|---------------|
| 2,800,442 | Brown   | July 23, 1957 |
| 2,978,391 | Du Rose | Apr. 4, 1961  |
| 3,006,822 | Todt    | Oct. 31, 1961 |

#### FOREIGN PATENTS

|         |               |               |
|---------|---------------|---------------|
| 858,718 | Great Britain | Jan. 11, 1961 |
|---------|---------------|---------------|

UNITED STATES PATENT OFFICE  
CERTIFICATE OF CORRECTION

May 12, 1964

Patent No. 3,133,006

Barnet D. Ostrow et al.

It is hereby certified that error appears in the above numbered patent requiring correction and that the said Letters Patent should read as corrected below.

Column 2, lines 9 and 10, formula (1) should appear as  
shown below instead of as in the patent:



Signed and sealed this 29th day of December 1964.

(SEAL)

Attest:

ERNEST W. SWIDER  
Attesting Officer

EDWARD J. BRENNER  
Commissioner of Patents